

FIP8309 OR 1,412,755

CATION OF TEXTILES &amp; FIBERS,

## UNITED STATES PATENT OFFICE.

NATHAN SINGER, OF NEWARK, NEW JERSEY, ASSIGNOR TO E. I. DU PONT DE NEMOURS &amp; COMPANY, OF WILMINGTON, DELAWARE, A CORPORATION OF DELAWARE.

## PROCESS OF TREATING BRISTLES.

1,412,755.

Specification of Letters Patent. Patented Apr. 11, 1922.

No Drawing.

Application filed September 4, 1918. Serial No. 252,615.

*To all whom it may concern:*

Be it known that I, NATHAN SINGER, of Newark, in the county of Essex, and in the State of New Jersey, have invented a 5 certain new and useful Improvement in Processes of Treating Bristles, and do hereby declare that the following is a full, clear, and exact description thereof.

My invention relates particularly to a 10 process for treating bristles, that is to say, the bristles obtained from animals, such as hogs, in which the bristles are treated in such a manner as to bleach them, and otherwise improve their value for commercial articles.

The object of my invention is to treat bristles, such for example, as hog bristles, in such a manner as to bleach them effectively, and by means of a process which 20 will cause the bristles to remain free from color after bleaching. Another object is to provide a process by means of which bristles of a very low grade and which are very yellow in color may be treated in such a way, 25 that they may be used to the same extent and to even greater advantage than high grade bristles that have been treated by previous processes. Another advantage is to treat bristles in such a manner that a 30

much greater proportion of the length of the bristle may be used in making up the bristles into commercial products, as for example, hair brushes. That is to say, by means of my process in treating the bristles, 35 it is not necessary to first remove the end of the bristle carrying the sack in which the bristle has grown, but the process is such as to almost entirely destroy the sack, thus making it possible to utilize this end of the 40 bristle without cutting, especially where, as in the case of hair brushes, the final trimming of the bristles in the brush will remove the ends which carry the sacks in the case of a certain proportion of the bristles.

45 The saving in the length of the bristle is also due to the fact, that my process effectively bleaches the bristle much closer to the end thereof which carries the "flag", so that a much shorter length of the bristles 50 is necessary to be removed at this end. As a consequence, the bristles treated in accord-

ance with my invention, may be used to make two separate lengths of bristles, that is to say, two separate bristles for insertion in a hair brush, whereas previously the length of the bristles was so reduced by cutting the two ends thereof, that only one bristle for insertion into a hair brush could be obtained from a single bristle in the raw state. Again, another advantage of my invention is the fact that the bristles resulting therefrom are much stronger, inasmuch as the ends carrying the sacks are retained. Again, my process results in giving the bristles a sheen, even in the case of low 65 grade Russian bristles, whereas formerly, such sheen was obtainable only in Japanese bristles. Furthermore, by leaving the sacks on the ends of the bristles, liquids applied to brushes made therewith, do not so readily 70 penetrate the canals of the bristles, and such bristles, therefore, dry much more quickly. Also, because of the fact that comparatively weak solutions are used in accordance with my process, the resulting bristles are less 75 brittle and less apt to be broken when folded for insertion into the brush backs.

Further objects of my invention will appear from the detailed description thereof contained hereinafter.

While my invention is capable of being carried out in many different ways, for the purpose of illustration I shall describe only certain ways of carrying out the same 85 herein.

For example, I may proceed as follows:

A quantity of the bristles, as for example, low grade Russian bristles is soaked in a solution containing peroxide of hydrogen for from ten to twelve hours. This solution 90 may be comprised of two and one-half gallons of three percent strength commercial hydrogen peroxide solution, made from barium peroxide, to which has been added one pound of sodium peroxide dissolved in 95 12½ gallons of water, and to which is added 11 fluid ounces of concentrated sulphuric acid. If necessary, the solution may be neutralized with ammonia to remove any excess of sulphuric acid. The bristles are 100 then washed with water. The treatment with this solution oxidizes the coloring mat-

ters, the materials of which the sacks are comprised, and the materials left by the sweat of the animal, thus giving the bristles a light blond color. Thereafter the bristles 5 are treated with a solution containing a hydrosulfite which may be obtained by adding from five to ten grams of zinc dust to 12 $\frac{1}{2}$  gallons of a solution made of 25% of sodium bisulphite solution of a strength of 10 35° Bé., and 75% of water. The bristles are left in this solution for 2 to 10 hours. Instead of the mentioned solution, I may use a solution of sodium bisulphite solution of a strength of 35° Bé., and 75% of water. 15 By this last treatment, the bristles are subjected to a reducing action which makes them practically colorless throughout the length of the same, down to a point very near to the end of the "flag", and which 20 gives them a very high lustre. The bristles are then again washed with water which may be slightly acidified with hydrochloric acid to remove the sodium salts which might otherwise crystallize upon the bristles. 25 While I have described my invention above in detail, I wish it to be understood that many changes may be made therein without departing from the spirit thereof.

I claim:—

- 30 1. The process of treating bristles which comprises subjecting the bristles to an oxidizing agent containing hydrogen peroxide.
2. The process of treating bristles which comprises subjecting the bristles to an oxidizing agent containing hydrogen peroxide, and then to a reducing agent.
- 35 3. The process of treating bristles which comprises subjecting the bristles to an oxidizing agent, and then to a reducing agent comprising a hydrosulfite acid.
- 40 4. The process of treating bristles which comprises subjecting the bristles to an oxidizing agent containing hydrogen peroxide, and then to a reducing agent comprising a hydrosulfite acid.
- 45 5. The process of treating bristles which comprises subjecting the bristles to an oxidizing agent, then washing the bristles, and then to a reducing agent comprising a hydrosulfite acid.
- 50 6. The process of treating bristles which comprises subjecting the bristles to an oxidizing agent containing hydrogen peroxide, then washing the bristles, and then to a reducing agent comprising a hydrosulfite acid.
- 55 7. The process of treating bristles which comprises subjecting the bristles to an oxidizing agent, then washing the bristles, then to a reducing agent comprising a hydrosulfite acid, and then again washing the bristles with water slightly acidified with hydrochloric acid.
- 60 8. The process of treating bristles which comprises subjecting the bristles to an oxidizing agent containing hydrogen peroxide, then washing the bristles, then to a reducing agent comprising a hydrosulfite acid, and then again washing the bristles with water slightly acidified with hydrochloric acid.
- 65 9. The process of treating bristles which comprises subjecting the bristles to an oxidizing agent containing hydrogen peroxide, then washing the bristles, then to a reducing agent comprising a hydrosulfite acid, and then again washing the bristles with water slightly acidified with hydrochloric acid.

dizing agent containing hydrogen peroxide, then washing the bristles, then to a reducing agent comprising a hydrosulfite acid, and then again washing the bristles with water slightly acidified with hydrochloric acid. 70

9. The process of treating bristles containing the bristle sacks which comprises subjecting the bristles to an oxidizing agent, then removing the flags and then cutting the bristles in the middle. 75

10. The process of treating bristles containing the bristle sacks which comprises subjecting the bristles to an oxidizing agent containing hydrogen peroxide, then removing the flags and then cutting the bristles in the middle. 80

11. The process of treating bristles containing the bristle sacks which comprises subjecting the bristles to an oxidizing agent, then to a reducing agent, then removing the flags and then cutting the bristles in the middle. 85

12. The process of treating bristles containing the bristle sacks which comprises subjecting the bristles to an oxidizing agent containing hydrogen peroxide, then to a reducing agent, then removing the flags and then cutting the bristles in the middle. 90

13. The process of treating bristles containing the bristle sacks which comprises subjecting the bristles to an oxidizing agent, then to a reducing agent comprising a hydrosulfite acid, then removing the flags and then cutting the bristles in the middle. 95

14. The process of treating bristles containing the bristle sacks which comprises subjecting the bristles to an oxidizing agent containing hydrogen peroxide, then to a reducing agent comprising a hydrosulfite acid, then removing the flags and then cutting the bristles in the middle. 100

15. The process of treating bristles containing the bristle sacks which comprises subjecting the bristles to an oxidizing agent, then washing the bristles, then to a reducing agent comprising a hydrosulfite acid, then removing the flags and then cutting the bristles in the middle. 110

16. The process of treating bristles containing the bristle sacks which comprises subjecting the bristles to an oxidizing agent containing hydrogen peroxide, then washing the bristles, then to a reducing agent comprising a hydrosulfite acid, then removing the flags and then cutting the bristles in the middle. 115

17. The process of treating bristles containing the bristle sacks which comprises subjecting the bristles to an oxidizing agent, then washing the bristles, then to a reducing agent comprising a hydrosulfite acid, then again washing the bristles with water slightly acidified with hydrochloric acid, then removing the flags and then cutting the bristles in the middle. 125

U.S. BLEACHING & DYEING; FLUID  
TREATMENT & CHEMICAL MODIFI-  
CATION OF TEXTILES & FIBERS,

U.S. PATENT OFFICE

1,412,755

3

18. The process of treating bristles containing the bristle sacks which comprises subjecting the bristles to an oxidizing agent containing hydrogen peroxide, then washing the bristles, then to a reducing agent comprising hydrosulphurous acid, then again washing the bristles with water slightly acidified with hydrochloric acid,

then removing the flags and then cutting the bristles in the middle. 10

In testimony that I claim the foregoing I have hereunto set my hand.

NATHAN SINGER.

Witnesses:

L. W. STETSON,  
LEON G. LORIMER.